# EUROPEAN PATENT SPECIFICATION

(11) **EP 0 463 136 B1**
(45) Date of publication and mention of the grant of the patent: **27.12.1995**
(21) Application number: 91901765.7
(22) Date of filing: 12.01.1991
(51) Int. Cl.: G03C 1/34, G03C 7/392

(54) **PHOTOGRAPHIC SILVER CHLORIDE EMULSIONS**
PHOTOGRAPHISCHE SILBERCHLORIDEMULSIONEN
EMULSIONS PHOTOGRAPHIQUES DE CHLORURE D'ARGENT

(30) Priority: 17.01.1990 GB 9001078
(43) Date of publication of application: 02.01.1992
(73) Proprietor: KODAK LIMITED, Harrow, Middlesex HA1 4TY (GB); EASTMAN KODAK COMPANY, Rochester, New York 14650-2201 (US)
(72) Inventor: LEYSHON, Llewellyn, James, Watford Herts. WD1 3HW (GB)
(74) Representative: Baron, Paul Alexander Clifford
(86) International application number: EP9100069
(87) International publication number: WO9110938

(56) References cited:
- WO-A-91/08515
- CHEMICAL ABSTRACTS, vol. 112, no. 4, 22 January 1990 Columbus, Ohio, USA S. Hirabayashi: "Silver halide color photographic material containing a magenta coupler of pyrazoloazole type and a bisphenol derivative to improve color quality" page 491

## Description

This invention relates to photographic silver chloride emulsions having improved keeping properties.

Photographic silver chloride emulsions are now widely used in the manufacture of photographic colour negative paper materials. As such materials age their sensitometric performance changes such that the speed and minimum density (Dₘᵢₙ) increase while their contrast decreases. Known techniques for countering these defects in silver halide emulsions in general include the method described in British Specification 1 262 127 which comprises the addition of small quantities of reducing agents such as amino- hexose-reductones. Control of the emulsion pH and pAg can also be beneficial.

There is, however, a need to improve the keeping properties (shelf life) of silver chloride emulsions still further.

Blocked bis-phenols have been described as photographic dye image stabilisers in European Patent specification 0 246 766 (US Patent 4 782 011). Specifically the compounds were incorporated into silver chlorobromide emulsions.

According to the present invention there is provided a method for improving the keeping properties of a silver chloride emulsion comprising at least 90% silver chloride which comprises incorporating therein a bisphenol derivative having two linked phenol rings wherein the hydrogen atom of one of the phenolic hydroxy groups is replaced by a blocking group which is a substituent other than hydrogen and at least one of the phenol rings is substituted.

The blocking group may be any group which does not affect the desired properties of the stabilizer.

The two phenol rings of the stabilizer may be linked directly by a single bond or indirectly by a linking group. Preferably, the link between the phenol rings is ortho relative to the phenolic hydroxy group of one ring and the blocked phenolic hydroxy group of the other ring.

Preferably, each phenol ring independently is substituted in a position ortho or para relative to the unblocked or blocked phenolic hydroxy groups. It is further preferred that substituents are present in both ortho and para positions.

The bis-phenol compound preferably has the general formula:
wherein
R is alkyl, cycloalkyl, alkenyl, aryl, acyl, alkylsuphonyl or arylsulphonyl,
R¹ is a single bond or a linking group selected from alkylene, alkylidene, a heteroatom or sulphonyl, and
each R² independently represents one or more substituents each selected from alkyl, alkoxy, alkenyl, cycloalkyl, aryl or aryloxy or, each R independently represents the atoms necessary to complete with the benzene ring to which it is attached, a fused polycyclic aromatic ring structure.
all of said alkyl, alkoxy, cycloalkyl, alkylene, alkenyl, aryl, aryloxy and acyl groups being optionally substituted.

Examples of blocking group R are methyl, ethyl, propyl or butyl, cyclohexyl, phenyl, acetyl or benzoyl.

Examples of linking group R¹ are methylene, butylidene, 3,5,5,-trimethylhexylidene, oxygen, sulphur or sulphonyl.

An especially preferred group of bis-phenol compounds has the general formula:
wherein R¹ and R are as defined above, and
R³, R⁴, R⁵ and R⁶ are each independently a substituted or unsubstituted alkyl, alkenyl, cycloalkyl or aryl group. Preferably, R₃ and R₄ are identical and R₅ and R₆ are identical.

Specific examples of bis-phenols suitable for use in the present invention are as follows:

The blocked bisphenol derivatives are readily prepared from their unblocked counterparts, many of which are commercially available. For example, a blocking group may be introduced into the unblocked parent bisphenol by reaction with an appropriate reactive halogen-containing compound e.g. an alkyl bromide, acyl chloride, sulphonyl chloride or a dialkyl sulphate e.g. diethyl sulphate.

Examples of unblocked parent bisphenols from which the stabilizers of the present invention may be prepared are as follows:

The present invention also provides a method for improving the keeping properties of a silver chloride emulsion comprising the incorporation therein of a bisphenol derivative having two linked phenol rings wherein the hydrogen atom of one of the phenolic hydroxy groups is replaced by a blocking group which is a substituent other than hydrogen and at least one of the phenol rings is substituted.

The silver chloride emulsions used in the present invention contain more than 90 mole %, silver chloride preferably the emulsions are substantially pure silver chloride.

The bis-phenol compounds may be incorporated in the silver chloride emulsions as a dispersion of droplets of a high boiling coupler solvent containing the bis-phenol. Such droplets may also contain a colour coupler. Alternatively they may be incorporated as solutions in an alcohol, for example, methanol.

The colour coupler may be of any class of couplers useful in colour photographic materials. Examples of such coupler classes include phenolic and naphtholic cyan couplers, pyrazolidone and pyrazolotriazole magenta couplers and acylacetanilide yellow couplers.

Particularly good results are obtained with the pivaloylacetanilide couplers and especially those with aryloxy coupling-off groups. Such couplers preferably have the general formula:
wherein
R⁷ represents one or more substituents of the type found in such couplers, and
R⁸ is a coupling-off group, preferably an aryloxy group.

Suitable emulsions, emulsion additives and couplers for use in the emulsions and elements of this invention are described in Research Disclosure, December 1978, Item 17643, published by Kenneth Mason Publications Ltd., 12a North Street, Emsworth, Hants PO10 7DQ, U.K. In particular, information on couplers and on methods for their dispersions are given in Sections VII and XIV, respectively, of this article.

The following examples are included for a better understanding of the invention.

### EXAMPLE 1

Four separate dispersions of the following coupler were prepared:
dissolved in one quarter its weight of dibutyl phthalate and 2-(2-butoxyethoxy)ethyl acetate. Two of the dispersions also contained a blocked bis-phenol as indicated below at concentrations equal to half that of the coupler, by weight. The fourth dispersion contained a comparison material the bis-phosphate ester of the formula:

(PhO)₂PO.O(CH₂)₁₀O.PO(OPh)₂

at the same concentration.

Each dispersion was mixed with a blue-sensitive silver chloride emulsion and coated on a resin-coated paper support, such that the silver and coupler coverages were, respectively, 0.18 g/m² and 0.40 g/m².

Strips of the fresh coatings were exposed and processed through RA4 chemistry to assess sensitometric performance. Further strips were incubated in the dark for 1 week at 50 °C and 50% RH before being similarly exposed and processed.

The Table below shows figures for the Dₘᵢₙ and contrast of the freshly coated and incubated strips from each coating. The columns labelled "Δ" show the difference between the fresh and incubated samples. Taking the coating without any addendum as a reference, the two blocked bis-phenols reduced the extent of Dₘᵢₙ increase and the loss in contrast due to incubation. A contrary effect was shown by the comparison bis-phosphate ester.

### EXAMPLE 2

Dispersions were prepared containing Compound I-11 with the colour couplers below:

Dispersions of each coupler alone were also made. In each dispersion the coupler was dissolved in its own weight of ethyl acetate and one half its weight of dibutyl phthalate. When present the bisphenol was included at half the weight of the coupler. The oil solutions were dispersed in aqueous gelatin using ultrasonic agitation as in Example 1.

Each dispersion containing Coupler (B) was mixed with a red-sensitised silver chloride emulsion and coated on a resin-coated paper support, such that the silver and coupler coverages were, respectively, 239 mg/m² and 425 mg/m². A second pair of coatings was made from the dispersions at the same component coverages but utilising a blue-sensitised emulsion (as used in Example 1) in place of the red sensitised emulsion.

Similarly the dispersions of Coupler (C) were coated together with a green sensitised silver chloride emulsion at silver and coupler coverages of 285 mg/m² and 447 mg/m² respectively.

Sample strips of the fresh coatings were exposed and processed through RA4 chemistry to assess sensitometric performance. Another strip from each coating was incubated in the dark for 8 days at 50°C and 50% RH before being exposed and processed.

The following table shows figures for the Dₘᵢₙ of the freshly coated and incubated strips. The column labelled "Δ" highlights the differences between the two sets, associated with the incubation treatment. All the coatings show an increase in Dₘᵢₙ on incubation and the magnitude of this increase is always reduced by the presence of the bisphenol.

The beneficial effect of the invention is thus shown not to be dependent on the colour sensitiviy of the emulsion or the coupler it contains.

## Claims

1. A method for improving the keeping properties of a silver chloride emulsion comprising at least 90% silver chloride which comprises incorporating therein a bisphenol derivative having two linked phenol rings wherein the hydrogen atom of one of the phenolic hydroxy groups is replaced by a blocking group which is a substituent other than hydrogen and at least one of the phenol rings is substituted.

2. A method as claimed in claim 1 in which the bisphenol derivative has the general formula: wherein
R is alkyl, cycloalkyl, alkenyl, aryl, acyl, alkylsuphonyl or arylsulphonyl,
R¹ is a single bond or a linking group selected from alkylene, alkylidene, a heteroatom or sulphonyl, and
each R² independently represents one or more substituents each selected from alkyl, alkoxy, alkenyl, cycloalkyl, aryl or aryloxy or, each R independently represents the atoms necessary to complete with the benzene ring to which it is attached, a fused polycyclic aromatic ring structure.

3. A method as claimed in claim 1 or 2 in which the bisphenol derivative has the general formula: wherein R¹ and R are as defined above, and
R³, R⁴, R⁵ and R⁶ are each independently a substituted or unsubstituted alkyl, alkenyl, cycloalkyl or aryl group.

4. A method as claimed in claim 3 in which R³ and R⁴ are identical and R⁵ and R⁶ are identical.

5. A method as claimed in any of claims 1-4 in which the emulsion comprises substantially pure silver chloride.

6. A method as claimed in any of claims 1-5 in which the emulsion further comprises a colour coupler.

7. A method as claimed in claim 6 in which the coupler is a yellow, cyan or magenta dye-forming coupler.

8. A method as claimed in claim 6 in which the coupler is an acylacetanilide, phenolic, naphtholic, pyrazolone or pyrazoloazole coupler.

## Patentansprüche

1. Verfahren zur Verbesserung der Aufbewahrungseigenschaften einer Silberchloridemulsion mit mindestens 90 % Silberchlorid, bei dem man in die Emulsion ein Bisphenol-Derivat einarbeitet, das zwei miteinander verbundene Phenolringe aufweist, wobei das Wasserstoffatom von einer der phenolischen Hydroxygruppen durch eine blockierende Gruppe ersetzt ist, bei der es sich um einen von Wasserstoff unterschiedlichen Substituenten handelt, und wobei mindestens einer der Phenolringe substituiert ist.

2. Verfahren nach Anspruch 1, bei dem das Bisphenol-Derivat die allgemeine Formel hat: worin bedeuten:
R gleich Alkyl, Cycloalkyl, Alkenyl, Aryl, Acyl, Alkylsulfonyl oder Arylsulfonyl,
R¹ eine einfache Bindung oder eine verbindende Gruppe, ausgewählt aus Alkylen, Alkyliden, einem Heteroatom oder Sulfonyl, und
R² jeweils unabhängig voneinander einen oder mehrere Substituenten, die jeweils ausgewählt sind aus Alkyl, Alkoxy, Alkenyl, Cycloalkyl, Aryl oder Aryloxy, oder worin R unabhängig voneinander steht für die Atome, die zur Vervollständigung einer an den Benzolring ankondensierten polycyclischen aromatischen Ringstruktur erforderlich sind.

3. Verfahren nach Anspruch 1 oder 2, bei dem das Bisphenol-Derivat die allgemeine Formel hat: worin R¹ und R die oben angegebene Bedeutung haben, und
R³, R⁴, R⁵ und R⁶ jeweils unabhängig voneinander stehen für eine substituierte oder unsubstituierte Alkyl-, Alkenyl-, Cycloalkyl- oder Arylgruppe.

4. Verfahren nach Anspruch 3, bei dem R³ und R⁴ identisch sind, und bei dem R⁵ und R⁶ identisch sind.

5. Verfahren nach einem der Ansprüche 1 bis 4, bei dem die Emulsion praktisch reines Silberchlorid aufweist.

6. Verfahren nach einem der Ansprüche 1 bis 5, bei dem die Emulsion weiterhin einen Farbkuppler enthält.

7. Verfahren nach Anspruch 6, bei dem der Kuppler ein einen gelben, einen blaugrünen oder einen purpurroten Farbstoff liefernder Kuppler ist.

8. Verfahren nach Anspruch 6, bei dem der Kuppler ein Acylacetanilid-, phenolischer, naphtholischer, Pyrazolon- oder Pyrazoloazolkuppler ist.

## Revendications

1. Procédé pour améliorer la conservation d'une émulsion au chlorure d'argent comprenant au moins 90 % de chlorure d'argent dans lequel on incorpore une dérivé de bisphénol ayant deux cycles phénol liés où l'atome d'hydrogène de l'un des groupes hydroxy phénolique est remplacé par un groupe bloquant qui est un substituant autre que l'hydrogène et l'un au moins des cycles phénol est substitué.

2. Procédé selon la revendication 1 dans lequel le dérivé bisphénol a la formule : où
R est alkyle, cycloalkyle, alcényle, aryle, acyle, alkylsulfonyle ou arylsulfonyle
R¹ est une liaison simple ou un groupe de liaison choisi parmi alkylène, alkylidène, un hétéro atome ou sulfonyle, et
chaque R² séparément représente un ou plusieurs substituants choisis parmi alkyle, alcoxy, alcényle, cycloalkyle, aryle ou aryloxy ou,
chaque R séparément représente les atomes nécessaires pour compléter avec le cycle benzénique auquel il est rattaché une structure aromatique polycyclique condensée.

3. Procédé selon la revendication 1 ou 2 dans lequel le dérivé bisphénol a la formule : où
R¹ et R sont tels que définis ci-dessus, et
R³, R⁴, R⁵ et R⁶ sont chacun séparément un groupe alkyle, alcényle, cycloalkyle ou aryle.

4. Procédé selon la revendication 3 dans lequel R³ et R⁴ sont identiques et R⁵ et R⁶ sont identiques.

5. Procédé selon l'une quelconque des revendications 1 à 4 dans lequel l'émulsion est pratiquement une émulsion pur chlorure.

6. Procédé selon l'une quelconque des revendications 1 à 5 dans lequel l'émulsion comprend de plus un coupleur chromogène.

7. Procédé selon la revendication 6 dans lequel le coupleur est un coupleur chromogène formateur de jaune, cyan ou magenta.

8. Procédé selon la revendication 6 dans lequel le coupleur est un coupleur acylacétanilide, phénolique, naphtolique, pyrazolone ou pyrazoloazole.
